

3,385,682

METHOD AND REAGENT FOR SURFACE  
POLISHING

Jack Lowen, Williamstown, Mass., assignor to Sprague Electric Company, North Adams, Mass., a corporation of Massachusetts  
No Drawing. Filed Apr. 29, 1965, Ser. No. 451,995  
2 Claims. (Cl. 51—293)

## ABSTRACT OF THE DISCLOSURE

A semiconductor polishing composition and process comprising applying to a semiconductor a carrying agent, a complexing agent, an oxidizing agent, and an abrasive material.

This invention relates to a method and reagent for polishing and preparing semiconductors, metals, and other materials for use in the electronics industry.

Semiconductors or other materials used in the electronics industry must have a smooth surface to effectively operate in their intended manner particularly in the latest planar structures. At present, many methods involving mechanical polishing or chemical polishing are employed with varying degrees of success to obtain the desired surface smoothness. These methods, however, are usually either too time consuming or too inefficient or yield surfaces marked by viscous fluid flow patterns.

An object of this invention is to provide a method and reagent for effectively polishing and preparing the surface of semiconductor crystals, combining the advantages of chemical and mechanical polishing.

In general, the reagent used in the method of this invention includes a complexing agent that can chelate with the material being polished, an oxidizing agent that can react with the material and an abrasive powder which are incorporated in a slurry using water or other media as a carrying agent. The slurry is applied to the material in a mechanical polisher such as Bausch & Lomb No. 21-11-86 enclosed in an air-tight box under a positive pressure of filtered air or inert gas such as nitrogen. A Sterilshield enclosure made by Baker is particularly effective.

The mechanical polisher used can be any standard mechanical polisher such as Bausch & Lomb No. 21-11-86 or Buehler Polishers or the new vibromatics put out by Fisher or Buehler. Prior to the polishing procedure a lapping schedule to remove all deformation caused by slicing or machining is essential. Regardless of how carefully the mechanical polishing operations are carried out, some surface deformation will remain. The incorporation of an active reagent to react with the material and a complexing agent to hold it in solution along with the usual abrasive slurry has a number of important advantages over either mechanical or chemical polishing:

(1) It is faster than mechanical polishing. Using versene and peroxide reduces the time necessary to polish silicon from about four hours to about one and one-half hours.

(2) Since the action is chemical as well as mechanical, the material abraded from the specimen reacts with the reagent and does not fill in scratches and imperfections on the surface as in mechanical polishing. A polished surface as produced by this method will have less surface damage than a mechanically polished surface.

(3) Since the action is mechanical as well as chemical, the sample is not marked by swirling patterns of hydraulic flow and the edges are not rounded to any significant dimension. The solutions used are not as corrosive or toxic and therefore safer for routine use.

The reagent of this invention is particularly effective

for polishing silicon, gallium-arsenide, germanium, and other semiconductors. The reagent or slurry of this invention attacks the surface to increase the rate of polishing, and dissolves the particles abraded from the material being polished to reduce abrasion and surface damage. Ordinarily, the polishing involves a surface smearing or film to cover and fill in surface damage. The slurry of this invention dissolves this film and produces a comparatively damage free surface.

10 The complexing agent used in the slurry may advantageously be selected from the following group:

|            |          |
|------------|----------|
| Versene    | chloride |
| fluoride   | citrate  |
| tartrate   | cyanide  |
| 15 oxalate | mannitol |

The oxidizing agent used in the slurry may advantageously be selected from the following group:

|            |             |
|------------|-------------|
| peroxide   | perchlorate |
| 20 nitrate | persulfate  |

or oxygen in the presence of hydroxide or perchlorate, etc. The abrasive material may be aluminum oxide or cerium oxide, diamond dust or other standard grinding or polishing powder.

25 The complexing agent is dissolved in water, or other suitable media, and filtered several times through hardened lint-free paper. This solution is generally stable and may be stored. Just prior to use the oxidizing agent is added and the solution re-filtered; the abrasive powder dispersed into the solution and the polisher loaded with the reagent slurry.

The reagent slurry generally contains the following components:

30 35 (a) complexing agent, 8 to 20% by weight  
(b) oxidizing agent, 1 to 10% by weight  
(c) abrasive, 20 to 80 g./250 ml. of slurry

40 The following are examples of specific applications of this invention:

## Example 1

Silicon or gallium arsenide is used as the semiconductor. The slurry contains the following components: one pound Versene (the tetrasodium salt of ethylene diamine tetra acetic acid) per gal. of H<sub>2</sub>O; approximately 3% of H<sub>2</sub>O<sub>2</sub>, i.e. 20-30 cc. of 30% per 250 ml. charge of slurry and 50-60 g. of Linde metallurgical Grade High Purity Alumina Abrasive.

## Example 2

45 Silicon is polished using 10 g. NaF, 5 g. NaOH, 50 ml. H<sub>2</sub>O<sub>2</sub>, 100 g. of Linde Metallurgical Grade Alumina and 25 ml. glycerine in 425 ml. H<sub>2</sub>O.

50 It is to be understood that the invention is not limited to the specific examples indicated above. For example, 5% KNO<sub>3</sub>, 5% KCl and 10% mannitol in a slurry containing 20% of Linde Metallurgical Grade Alumina can be used to polish germanium.

55 Since it is obvious that many changes and modifications can be made without departing from the nature and spirit of the invention, it is to be understood that the invention is not limited to the above description except as set forth in the appended claims.

What is claimed is:

60 65 1. A reagent slurry for surface polishing a semiconductor consisting essentially of from 8 to 20% by weight of a member of the group consisting of the tetrasodium salt of ethylene diamine tetra acetic acid, sodium fluoride and mannitol; 1 to 10% by weight of a member of the group consisting of hydrogen peroxide and potassium nitrate; a carrying agent selected from the group consisting of water and a water and glycerine mixture; and from

20 to 80 g./250 ml. of slurry of a hard abrasive selected from the group consisting of aluminum oxide, cerium oxide and diamond dust.

2. A method of polishing the surface of a semiconductor comprising applying the composition of claim 1 to the surface of said semiconductor while maintaining relative motion between said semiconductor and said composition.

**References Cited**

UNITED STATES PATENTS

1,800,881 4/1931 Andrus et al. ----- 106—14  
2,082,950 6/1937 Green ----- 106—14

|           |         |                       |            |
|-----------|---------|-----------------------|------------|
| 2,294,760 | 9/1942  | Morris -----          | 51—307     |
| 2,683,343 | 7/1954  | Gillette et al. ----- | 51—304     |
| 3,103,733 | 9/1963  | Fauro et al. -----    | 204—143    |
| 3,158,517 | 11/1964 | Schwarzenberger --    | 252—79.3 X |
| 3,228,816 | 1/1966  | Kendall -----         | 204—140.5  |
| 3,248,235 | 4/1966  | Pryor et al. -----    | 51—304     |

**OTHER REFERENCES**

Camp, A Study of the Etching Rate of Single-Crystal Germanium, Journal of Electro-Chem. Society, vol. 102, Nov. 10, 1955, pp. 586—593.

DONALD J. ARNOLD, *Primary Examiner.*